

Z. JEFFRIES AND W. A. GIBSON,

ALLOY.

APPLICATION FILED JULY 30, 1919.

1,352,271.

Patented Sept. 7, 1920.



Inventors

Zay Jeffries  
by and Wm A. Gibson  
Ray J. Lehr  
attorney

# UNITED STATES PATENT OFFICE

ZAY JEFFRIES AND WILLIAM A. GIBSON, OF CLEVELAND, OHIO, ASSIGNORS TO THE ALUMINUM CASTINGS COMPANY, OF CLEVELAND, OHIO, A CORPORATION OF OHIO.

## ALLOY.

1,352,271.

Specification of Letters Patent. Patented Sept. 7, 1920.

Application filed July 30, 1919. Serial No. 314,261.

To all whom it may concern:

Be it known that we, ZAY JEFFRIES and WILLIAM A. GIBSON, citizens of the United States, residing at Cleveland, in the county 5 of Cuyahoga and State of Ohio, have invented certain new and useful Improvements in Alloys, of which the following is a specification, reference being had therein to the accompanying drawing.

10 This invention relates to improvements in aluminum alloys and is concerned especially with aluminum alloys containing zinc, copper and iron.

One object of the invention is to provide 15 an aluminum alloy containing zinc having physical properties, especially tensile strength and ductility, superior to those possessed by aluminum-zinc alloys heretofore known.

20 Another object of the invention is to provide an aluminum-zinc alloy having superior physical properties in combination with ease of preparation and good casting, machining and working qualities.

25 Binary alloys of aluminum and zinc have been extensively investigated and it has long been known that the effect of zinc when added to aluminum is to produce relatively close grained and non-porous castings. By many it has been supposed that 30 these aluminum-zinc alloys essentially are subject to excessive corrosion and offer relatively slight resistance to shock. It is now known, however, that these objectionable 35 characteristics are entirely obviated when suitable care is taken to insure uniform mixing of the constituent metals in proper proportions.

The ternary alloys of aluminum, zinc and 40 copper have been only slightly investigated so far as we are aware. Their physical properties, however, so far as known, are appreciably better than those of the binary aluminum-zinc alloys. We have found that 45 an aluminum alloy containing about 8% zinc and 3% copper has a tensile strength ranging from 20,000 pounds to 26,000 pounds per square inch, and an elongation of from 3% to 4%. (Here, as elsewhere in 50 this application, the composition percentage is by weight).

We have discovered that these physical properties can be very greatly improved by the addition to a ternary alloy of the above

composition of from 0.5% to 1.5% of iron. 55 While the proportions of the various constituents may vary through a considerable range and still retain in substantial measure the advantages of this four part alloy, the composition which we prefer to employ 60 is one containing from 6% to 8% zinc, from 2.5% to 3.5% copper, from 1% to 1.5% iron, and the remainder aluminum. Alloys within this range of composition, when cast in ordinary green sand, have tensile strengths 65 ranging from 24,000 pounds to 30,000 pounds per square inch, elastic limits ranging from 15,000 pounds to 17,000 pounds per square inch, elongations of from 5% to 6%, Brinell hardness numbers ranging 70 between 55 and 60, and specific gravities less than 3.0. By increasing the percentage of zinc and decreasing that of aluminum greater tensile strength is obtained but at the sacrifice of ductility. 75

An alloy of the preferred composition can be made up in various ways known to those skilled in the art. One successful method is as follows:

First is prepared a rich alloy containing 80 three parts of copper to one part of iron together with a sufficient amount of aluminum to reduce the melting point of the alloy to approximately that of aluminum. The calculated amounts of aluminum and 85 of the above rich alloy are melted together and the calculated quantity of zinc is then added while stirring. After thorough stirring the metal is heated to the desired pouring temperature. This alloy may be cast 90 equally well in sand molds and permanent molds and by reason of the zinc content, which renders the melt quite fluid, it will completely and quickly fill the mold, even where there are thin sections. The alloy 95 is easy to make because no extremely high temperatures are required. Castings of this alloy are very dense, have good machining qualities and are not easily corroded or affected by shocks. 100

We have found that it is not advantageous to heat treat these alloys, for while heat treatment may in some cases increase tensile strength somewhat, it results in a relatively greater decrease of the elastic 105 limit. For most purposes the lowering of the elastic limit would outweigh the advantages incident to any increased tensile

strength so that, as stated, heat treatment of the alloy is not ordinarily advantageous.

The accompanying drawing shows graphically the tensile strength and elongation (a) of aluminum alloys with 3% copper and varying amounts of zinc and (b) of aluminum alloys with 3% copper, varying amounts of zinc and 1% added iron. The broken line curves represent the alloys with-  
10 out iron and the full line curves represent the alloys with iron. The horizontal scale at the bottom represent the per cent. of zinc, the vertical scale at the left, tensile strength and the vertical scale at the right, the per  
15 cent. elongation. It will be observed that the addition of 1% iron to the ternary alloy markedly increases both the tensile strength and the elongation. With 7% to 8% zinc the alloy presents a highly advantageous  
20 combination of tensile strengths ranging from over 27,500 pounds to over 28,500 pounds per square inch and elongation ranging from over 6% to over 7%, whereas the ternary alloy without the iron has a tensile  
25 strength ranging well below 24,000 pounds per square inch and an elongation ranging well below 4%.

As has already been indicated, if the use of the alloy requires a still higher tensile  
30 strength this can be obtained at the sacrifice of ductility, by increasing the quantity of zinc above, say 8%, and maintaining the iron and copper contents. However, these aluminum alloys containing more than 8%  
35 zinc with 1% iron and 3% copper are not only stronger but also more ductile than the aluminum alloys containing zinc and copper alone. For example, as will be noted on reference to the drawing, with 15% zinc and  
40 3% copper and 1% added iron the tensile strength is 37,000 pounds per square inch, and elongation 2.5% whereas the same composition without the iron has a tensile strength of 32,000 pounds per square inch  
45 and an elongation of 1.8%.

As is well known to those having commercial experience with aluminum, it is impossible to secure the metal in commercial quantities free from impurities, notably iron  
50 and silicon. The iron thus present will, of course, be taken account of in introducing additional iron; and care should be taken

to keep the amount of silicon present as low as possible.

It may be observed in connection with the 55 values mentioned for tensile strength and ductility, that in the case of castings made from our improved alloy the tensile strengths increase and the ductility decreases slightly as the castings age.

In the foregoing description we have indicated the preferred range of compositions and the preferred method of preparing our improved alloy, but it is to be understood that our invention is not limited in these respects except as specified in the appended 60 claims.

What we claim is:

1. An alloy containing aluminum, copper, zinc and iron, the copper content being 70 from 2% to 5%, the zinc content being from 4% to 25%, the iron content being from 0.6% to 1.8%, and the aluminum making up the remainder.

2. An alloy containing aluminum, copper, zinc and iron, the copper content being from 2% to 5%, the zinc content being from 4% to 16%, the iron content being from .6% to 1.8%, and the aluminum making up 75 the remainder.

3. An alloy containing aluminum, copper, zinc and iron, the copper content being from 2.5% to 3.5%, the zinc content being from 6% to 8%, the iron content being from 0.8% to 1.5%, and the aluminum making up 80 the remainder.

4. An alloy of aluminum, copper, zinc and iron containing approximately 88.7% aluminum, 3% copper, 1.3% iron and 7% zinc.

5. An alloy containing aluminum, copper, zinc and iron, the copper content being approximately 3%, the iron content being approximately 1.3% and the zinc content ranging from 4% to 25%, and the aluminum 95 making up the remainder.

6. An alloy containing aluminum, from 2% to 5% of copper, from .5% to 1.5% of iron and zinc and having a specific gravity less than 3.0.

In testimony whereof, we hereunto affix our signatures.

ZAY JEFFRIES.  
WILLIAM A. GIBSON